

Jan. 8, 1929.

1,697,920

K. KOLLER

PROCESS OF MAKING PRODUCER GAS FROM COKING COALS

Filed July 18, 1925



INVENTOR.  
K. Koller  
BY Marks & Clark  
ATTORNEYS.

Patented Jan. 8, 1929.

1,697,920

# UNITED STATES PATENT OFFICE.

KARL KOLLER, OF BUDAPEST, HUNGARY.

## PROCESS OF MAKING PRODUCER GAS FROM COKING COALS.

Application filed July 18, 1925, Serial No. 44,625, and in Germany July 18, 1924.

This invention relates to certain improvements in the process of gasification of coking coals in gas producers.

As known, coals which cake together can not readily be completely gasified in the generator by reason of the caking and swelling of the coal at certain temperatures, whereby also a great amount of mechanical labor is necessary to maintain the layer or column of coal permeable.

It is known that these coals may be dry distilled without their coking together if the temperature is held so low (below 500° C.) that conversion (cracking) of the resulting tar distillates and colloids does not take place. Colloids can, however, separate out in certain kinds of coal even at low temperature. These colloids cause caking of the coal. In such cases the coal may lose its capacity for caking together or coking, by preliminary oxidation of this tar constituent (colloids) at low temperature (below 200° C.).

These coals have such a high carbon content that gasification thereof causes reactions involving high temperatures, and the temperature of the gases passing off from the gasifying zones lies far above this so-called crackling temperature, and this is so even in the case when a mixed gas with too high a hydrogen content is produced.

Most industries operating with producer gas, for example, the iron, ceramic, glass industries, lime works, etc. desire a gas, rich in carbon monoxide, so that the addition of steam must not exceed certain limits.

The present invention is directed to a process for the complete gasification of coking coals in a gas producer, by introducing gases arising from a point outside the producer, in which the temperature in the distilling zone of the gas generator is held constantly below the crackling temperature of the tar products, in that the heat resulting from the exothermic reactions is modified by the endothermic reaction of the foreign gases introduced. By means of these endothermic reactions the temperature in the combustion zone, that is, in the first zone above the grate, the gasifying zone proper and the temperature of the gases rising from the gasifying zone, is reduced to such degree that the distilling temperature may correspond to the above conditions.

The heat-combining foreign gases may be chiefly the gases rich in CO<sub>2</sub> from various furnaces (for example, combustion gases).

The reduction of the CO<sub>2</sub> is the most active endothermic reaction and gas which is rich therein is always available in large quantities. By regulating the quantities of gas supplied it is possible to regulate the temperature of the gases issuing from the gasification zone according to the type of coal to be gasified.

The foreign gases may suitably be introduced together with the air-steam mixture under the grate, so that the fan sucks in air as well as foreign gas, and the combination of the mixture drawn in regulated by suitable regulating devices, such as slides, dampers, etc. The combination or composition of the mixture may be constantly controlled by means of a suitable gas tester.

The process of the application also consists in that in those types of coal which give colloids even at low temperature distillation, and thus produce coking as a result of such low temperature distillation, in addition to being supplied with the gas mixture (air, steam, and gases containing carbon dioxide) below the grate, oxygen or air is supplied to the distilling chamber, for the purpose of oxidizing those colloids which separate out at low temperature distillation, and thus prevent the coals from caking. In this process the temperature in the distilling chamber is maintained below the ignition temperature and care must be observed that only so much oxygen is introduced into the distilling chamber that an explosive gas cannot form.

The figure illustrates an apparatus in vertical section for carrying out the above process. The gas producer is charged with fuel via a charging hopper 2. The fuel is distilled in a distillation zone 3 and gasified in a gasifying zone 4 by means of air and steam entering pipe 5 and nozzle 6. To this air and steam mixture is added the required quantity of CO<sub>2</sub> or any other gas capable of regulating the process before entering the producer. Ashes are removed via pan 7; additional air or oxygen may be admitted to the distillation chamber via the conduit 8 and valve 9 to oxidize the colloidal constituents of the coal.

Having now described my invention, I claim:

1. In the process of making producer gas from the total gasification of coal in a gas producer having a distilling zone and a gasification zone, the steps which comprise, admitting regulated quantities of mixed air, steam and carbon dioxide to the gasification

zone to generate producer gas, passing the hot producer gas through the distilling zone to distill and gasify coal therein, and simultaneously introducing a limited and regulated supply of oxygen directly into the distilling zone to oxidize colloidal constituents of the coal and thereby prevent caking of the coal of the distilling zone.

2. In the process of making producer gas from the total gasification of coal in a gas producer having a distilling zone and a gasification zone, the steps which comprise, admitting regulated quantities of mixed air, steam and carbon dioxide to the gasification zone

to generate producer gas, passing the hot producer gas through the distilling zone to distill and gasify coal therein, and simultaneously introducing a limited and regulated supply of oxygen directly into the distilling zone to oxidize colloidal constituents of the coal and thereby prevent caking of the coal in the distilling zone, the temperature of the distillation zone at the point of introduction of the oxygen being maintained below the ignition temperature of the gases at that point.

In testimony whereof I have signed my name to this specification.

KARL KOLLER.